

## UNITED STATES PATENT OFFICE.

ROBERT JOHN, OF NEW YORK, N. Y., ASSIGNOR TO DAYLIGHT FILM CORPORATION, A CORPORATION OF NEW YORK.

## COMPOSITION OF MATTER FOR PHOTOGRAPHIC PROCESSES.

No Drawing. Original application filed May 6, 1916, Serial No. 95,957. Divided and this application filed July 25, 1919. Serial No. 313,236.

To all whom it may concern:

Be it known that I, ROBERT JOHN, a citizen of the United States, residing at New York, in the county of New York and State of New York, have invented a certain new and useful Composition of Matter for Photographic Processes, of which the following is a specification.

My invention relates to a composition of matter for photographic processes and has for its object to produce a printing surface containing a photographic record of lights and shades from which copies can be made by a dye or ink contact transfer process. 10 An illustrative dye contact transfer process is disclosed in patent to Shepherd and Bartlett No. 728,310, granted May 19, 1903, for photographic printing, and an illustrative ink contact transfer process is disclosed 15 in Cassell's Cyclopaedia of Photography, Cassell & Co., New York, 1912, at page 124 under the title "Collotype", it being understood, however, that the processes thus illustrated do not disclose a printing plate having 20 the novel and beneficial characteristics of the printing plate obtained by the use of the composition of matter disclosed and claimed herein. Although the preferred method is to obtain the photographic record 25 for the printing surface from a completed negative, it may be obtained by direct exposure, as, for example, in a camera, the details of which method are disclosed in a pending application for Letters Patent 30 Serial No. 327,890, filed October 2, 1919, for process of photographic reproduction directly from a negative. The printing surface when treated with dye or ink also may be used in the same manner as a positive, 35 either for direct view, or with reflected light, or with transmitted light as in a projecting machine.

This application is a division of my co-pending application for Letters Patent 40 Serial No. 95,957, filed May 6, 1916, for photography.

The invention is applicable to monochromatic, polychromatic, or natural color photography both in still photography and 45 in motion picture photography. The term "color" is intended to include "black", which sometimes technically is designated as an absence of color.

In the embodiment of my invention chosen for purposes of illustration, a sensitized emulsion such as a silver salt emulsion is exposed to the action of light modified by the lights and shades of the completed negative which it is desired to reproduce. The silver salt emulsion may be carried or mounted on any desired support, 55 either opaque, translucent, or transparent, but preferably is mounted on a transparent carrier such, for example, as glass or a cellulose base, in order that the silver salt emulsion may be exposed to the modified light through its transparent carrier.

The emulsion then is treated by a developing solution containing a hardening or tanning agent which hardens or renders insoluble or unremovable the emulsion adjacent its light affected, light sensitive content, the effect of which agent is controlled or limited selectively by the presence of varying quantities of a neutralizing agent, 70 after which the unhardened or soluble or removable portions of emulsion are removed in any desired manner, as, for example, by melting with warm water.

The result of the above treatment is the 80 production of what may be termed a printing surface having novel characteristics and beneficial properties never before attained.

The most important of the novel characteristics is a printing or reproducing surface comprising granules or great numbers of photographically formed, extremely minute, individual protuberances which are distributed and grouped irregularly so as 85 to represent photographic lights and shades.

The most important of the beneficial properties is that such a printing surface when treated with a dye, ink, or other coloring matter, will absorb or take up or 90 carry the coloring matter within a few seconds, and when thus treated and placed in contact with a substance which is to carry the final reproduction, such for example as a gelatin, will give up its coloring matter 95 practically instantaneously and produce on said gelatin an exact and perfect reproduction. This speedy result, which is novel and was impossible of attainment before the present invention, is of prime importance 100 in the production of motion picture posi-

tives from motion picture negatives, although the saving of time and the superior results obtainable in still photography also are important. The printing plate or film, moreover, when treated with coloring matter, may be used as a positive if reproductions are not desired.

A sample formula for a developing solution containing a hardening or tanning agent the effect of which is controlled and limited selectively by the presence of varying quantities of a neutralizing agent is as follows:

|    |                   |               |
|----|-------------------|---------------|
| 15 | Water             | 8.5 ozs.      |
|    | Pyrogallic acid   | 11 grs.       |
|    | Metol             | 9 grs.        |
|    | Potassium bromide | 4 grs.        |
| 20 | Sodium carbonate  | 200 grs.      |
|    | Sodium sulphite   | 40 to 60 grs. |

In the above sample formula the hardening or tanning agent is pyrogallic acid, and the controlling and limiting agent is sodium sulphite which may be varied in amount selectively within limits to obtain the desired result. It is well known that pyrogallic acid also is a developing agent and that sodium sulphite is a preservative adapted to prevent oxidation of the pyrogallic acid in solution. Other hardening and tanning agents and other neutralizing agents may be used, the above formula representing one developing solution by which the process may be carried out. Potassium bromide, for example, also has a certain controlling and limiting effect. The main difference between the above sample formula and standard developing formulas is in the amount of sodium sulphite used. In standard formulas the amount of sodium sulphite used is so greatly in excess of the amount used in the above sample formula that the tanning or hardening effect of the pyrogallic acid is entirely neutralized or overcome. In the sample formula, the sodium sulphite merely controls and limits the hardening effect of the pyrogallic acid. It is of course understood by those skilled in the art that when a thick layer of emulsion is treated, or when the exposure is through the transparent carrier, it is advisable, in order to accelerate the action of the pyrogallic acid, to use larger quantities of an accelerator such, for example, as sodium carbonate or its equivalents than when the emulsion layer is thin or exposed on its face. When larger quantities of sodium carbonate thus are used, it is necessary to increase the amount of sodium sulphite. The above sample formula is for treatment of an emulsion exposed through its transparent carrier and therefore contains a comparatively large amount of sodium carbonate with an increased amount of sodium sulphite. In order to obtain the de-

sired printing surface, however, the amount of sodium sulphite in the process disclosed herein is much less than would be used in a developing solution for the usual development of the particular emulsion layer to be treated. Although it is preferable for reasons of convenience to embody the selectively controlled hardening agent in the developer solution, it may be used separately if desired, by such modification of the developer solution as will prevent such a hardening of the emulsion as will prevent the selective hardening desired.

It is believed that the hardening or tanning effect of the pyrogallic acid exerts its action first adjacent the so-called latent image, or in other words, on the portions of emulsion adjacent the particles of silver salts affected by the exposure light and converted by the developer into metallic silver. Thus in a silver bromide film, the throwing off of the bromide from a light affected silver bromide particle in the developing process, probably reacts with the pyrogallic acid to harden or tan or render insoluble or unremovable the adjacent emulsion. Thus in the embodiment chosen for purposes of illustration, the reaction products from the chemical effects of the developer solution, are believed to react with the selectively controlled hardening agent. However this may be, it is necessary for purposes of my invention only either to harden particles of emulsion adjacent light affected particles of the light sensitive content in any desired manner, or in reverse manner to leave unhardened the particles of emulsion adjacent light affected particles of the light sensitive content and harden the remaining emulsion, the essential result being a hardened emulsion surface corresponding to the lights and shades to be reproduced which will acquire and give up any desired color in a comparatively short time. By controlling the hardening or tanning effect of the pyrogallic acid as above set forth, only the particles of emulsion adjacent the said light affected particles of silver salts are hardened, the relative proportions of the hardening agent (whether or not accelerated by an accelerating agent) and of the neutralizing agent being such as to control selectively the effective area of influence of the hardening agent. The unhardened portions, as stated above, then may be removed in any desired manner as by placing the emulsion in warm water which causes the unhardened or soluble portions to soften and melt away from the hardened or insoluble portions so that the hardened emulsion alone will remain in the form of extremely minute, individual protuberances which are distributed and grouped irregularly so as to represent the photographic lights and shades which it is desired to reproduce. It is preferable that

only those portions of emulsion be hardened which are adjacent the carrier for the emulsion, which may be accomplished in various ways, some of which are disclosed in my co-pending applications for Letters Patent Serial No. 313,239, filed July 25, 1919, for a thin mounted sensitized emulsion; Serial No. 313,240, filed July 25, 1919, for process of making a contact transfer printing surface by complementary light; Serial No. 327,891, filed October 2, 1919, for potassium iodide formula for photographic processes, process of using same, and article obtained thereby; Serial No. 332,806, filed October 15, 1919, for process of making a contact transfer printing surface with a colored emulsion, and among which may be mentioned the exposure of the sensitized emulsion through its transparent carrier and the limitation of the depth to which the rays of exposure light penetrate by having the actinic rays of the exposure light and the emulsion complementary in color.

If desired the hardened emulsion may be fixed to remove the silver salts unaffected by light, and bleached to remove the black metallic silver. This may be done in well known manner, and while not necessary, is of advantage as it enables the operator to watch the effect of the coloring matter on the printing surface to which it is applied for carrying out the printing process.

The order of melting, bleaching, and fixing is not important and may be carried out in any order desired, although it generally is more convenient to fix, melt, and bleach, in the order named.

The printing of positives from the printing surface may be done by direct contact. The printing surface is exposed to the action of the desired coloring matter as by placing it in or carrying it through a liquid color bath. The colored surface then is placed in contact, preferably under some pressure, with the substance on which the positive is to be made, as by a roller by a squeegee action. As stated above, the printing surface prepared by my process receives and gives up the coloring matter almost instantly as distinguished from other processes which take an appreciable length of time.

Natural color effects may be produced in well known manner, such for example as by exposure through color screens with subsequent treatment and manipulation to obtain the desired results.

Many modifications of my invention will be apparent to those skilled in the art without departing therefrom or from the scope of the claims, my invention not being limited to the embodiments thereof chosen for purposes of illustration but consisting of a composition of matter for forming a printing surface capable of acquiring and giving up a desired color with great rapidity.

By the term "metol" in this case is meant monomethylparamidophenol sulphate or its equivalents.

Having described one embodiment of my invention, what I claim is:

1. A developing and hardening composition of matter containing an emulsion hardening and silver salt developing substance and a substance partially but not entirely neutralizing the emulsion hardening effect of said developing and hardening substance in such amount as to permit only a selective area of hardening.

2. A developing and hardening composition of matter containing pyrogallic acid and a substance partially but not entirely neutralizing the emulsion hardening effect of said pyrogallic acid in such amount as to permit only a selective area of hardening.

3. A developing and hardening composition of matter containing pyrogallic acid and sodium sulphite in which the amount of sodium sulphite is sufficient only to control but not eliminate the hardening effect of the pyrogallic acid.

4. A gelatin hardening composition of matter containing an emulsion hardening substance and a substance partially but not entirely neutralizing the emulsion hardening effect of said hardening substance in such amount as to permit only a selective area of hardening.

5. An emulsion hardening composition of matter containing pyrogallic acid and a substance partially but not entirely neutralizing the emulsion hardening effect of said pyrogallic acid in such amount as to permit only a selective area of hardening.

6. A developing and hardening composition of matter containing water, pyrogallic acid, metol, potassium bromide, sodium carbonate, and sodium sulphite in which the amount of sodium sulphite is sufficient only to control but not eliminate the hardening effect of the pyrogallic acid.

7. A developing and hardening composition of matter containing

|                   |               |     |
|-------------------|---------------|-----|
| Water             | 8.5 ozs.      | 115 |
| Pyrogallic acid   | 11 grs.       |     |
| Metol             | 9 grs.        |     |
| Potassium bromide | 4 grs.        |     |
| Sodium carbonate  | 200 grs.      |     |
| Sodium sulphite   | 40 to 60 grs. | 120 |

8. A developing and hardening composition containing pyrogallic acid, sodium sulfite and sodium carbonate, in which the sulfite is present only in sufficient quantity to control but not eliminate the hardening effect of the pyrogallic acid.

9. A developing and hardening composition containing pyrogallic acid, sodium sulfite and sodium carbonate, in which the ratio by weight on the dry basis, of carbon-

ate to sulfite is greater than 3:1 and in which the sulphite is present only in sufficient quantity to control but not eliminate the hardening effect of the pyrogallic acid.

10. A developing and hardening composition containing pyrogallic acid, sodium sulfite and sodium carbonate, in which the ratio by weight, on the dry basis, of carbonate to pyrogallic acid is about 10:1

and in which the sulphite is present only in sufficient quantity to control but not eliminate the hardening effect of the pyrogallic acid.

In testimony that I claim the foregoing, I have hereunto set my hand this 23rd day <sup>15</sup> of July, 1919.

ROBERT JOHN.